

July 21, 1942.

B. HORSFIELD

2,290,686

TREATMENT OF MATERIAL PARTICLES

Filed May 26, 1939



Basil Horsfield

INVENTOR

By *Freeman, Scott, Elbert, and Widman*

ATTORNEYS

## UNITED STATES PATENT OFFICE

2,290,686

## TREATMENT OF MATERIAL PARTICLES

Basil Horsfield, Pittsburgh, Pa., assignor to Edwin  
L. Wiegand, Pittsburgh, Pa.

Application May 26, 1939, Serial No. 275,961

19 Claims. (Cl. 209—2)

My invention relates to the treatment of material in the form of particles, to remove foreign material of slime nature, either co-mingled with the particles or adhering to the particles, and, more particularly to remove objectionable coatings from the individual particles, and the principal object of my invention is to provide a new and improved method of such treatment.

One material to which my method may be applied is zircon sand or ore. The particles of this material often are found to have films or coatings of iron oxide or some other foreign material or combination of foreign materials. These coatings are usually in the form of a more or less complete shell surrounding the individual particle. These foreign materials are objectionable, particularly if the zircon is to be used as electrical insulating material, for example. A very small amount of such foreign material will make a very great difference in the resistivity of a mass of insulating material, particularly if the material is subjected to elevated temperatures. While zircon has been given as an example, it will be understood by those skilled in the art that my invention may be applied in connection with other similar insulating materials, or other materials.

In the single figure of the drawing accompanying this specification, and forming a part of this application, I have shown, for purposes of illustration, one embodiment of my invention in more or less diagrammatic form.

The material to be treated in accordance with my invention may be first subjected to preliminary treatment such as rough screening, screening to size, magnetic separation, soaking, washing, and so forth, as may be desired or considered necessary in connection with the particular material.

The material, preliminarily treated or not, as the case may be, is introduced into a hopper 10 through a conduit 11, or in any other suitable way. The hopper 10 has an outlet 12 suitably connected, as by a pipe 13, with the feed end of a rotary tumbling barrel or mill 14, this mill being here shown, diagrammatically, as of the type commercially known as a Hardinge conical ball mill. It is desired that the material be treated in the mill 14 in the presence of water, and, if the material fed into the hopper 10 is not already mixed with water, water may be fed into the hopper 10 by a conduit 15, or otherwise fed to the material. In practicing my method it is preferred that the mill 14 contain no balls or other like grinding bodies as it is not

desired that the particles be ground to greater fineness, but that the undesirable coatings be scuffed therefrom. The desired scuffing action is produced by self-attrition, that is, by movement of the surface of a particle upon the surface of another particle. Such movement is caused by the rotation of the mill 14 and resultant tumbling of the material. In the mill 14, the material more or less settles from the liquid in the mill, thus increasing the rubbing or scuffing action as the mill rotates.

It will be understood that the speed of the mill will control to some extent the nature of the scuffing action. The speed should not be high enough to lift the material through an arc of 180° but should turn the load on itself somewhat below this angle. For a gentle attrition 10 R. P. M. is desirable but speeds up to 40 R. P. M. or more may be used depending somewhat upon 15 the nature of the material being treated and the size of the mill. In the case of treating zircon, it is desired to remove any coating of foreign material and not to abrade the crystal surface but scuff it clean. For this material, I have 20 found in medium size conical mills of 4 feet diameter or larger, that from 10 to 20 R. P. M. is a desirable operating speed. The time of milling 25 is also important. I have found that, in the treatment of zircon to be used for electrical purposes, a time of from 4 to 6 hours is desirable. However, the time may be greatly extended, particularly if the mill is operated at a very low 30 speed, or the time may be shortened to an hour or somewhat less, depending upon the particular material to be treated, the speed of the mill, and the results desired. I have found that even 35 a small amount of self-attrition produced in the mill produces a material which gives results which are measurably better than a material 40 which has not been so treated.

It will be understood that the material may be treated in the mill 14 as a batch for the desired period of time, or material may be continuously fed into the mill and continuously discharged therefrom, in which case the dwell in 45 hours, of the material in the mill, is on the average equivalent to the charge carried by the mill continuously, divided by the hourly feed rate in filling the mill.

50 Preferably, a basic solution is fed to the material to be treated at a suitable and desired place, or places. A receptacle 16 containing such a solution is here shown as connected by a pipe 17 through a valve 18 to the hopper 10, enabling 55 a small quantity of the basic solution to be added

to the material in the hopper 10, and hence to the material in the mill 14, and to the material in a separator, as will appear. The basic solution may be added continuously in accordance with continuous feed of material through the pipe 13 to the mill 14.

I have found that with an acid solution, that is, a solution where pH is less than 7, in the mill 14, the scuffings, though mechanically separated from the particles by the action in the mill, tend to cling to the particles, probably due to an electrostatic effect, thereby hindering a separation of the particles from the scuffings. On the other hand, I have found that in a basic or neutral solution the scuffings do not cling to the particles but are in suspension in the liquid. Desirably, the hydrogen ion concentration of the solution in the mill 14 is made such that pH is equal to 8 or more. Ammonium hydroxide may be used as the basic material, and this material has the further advantage of being a dispersing agent of high basicity, as well as being completely volatile without residue, but any other suitable material may be utilized.

The material treated in the mill 14 is discharged therefrom through a conduit 19 to the feed end of a washer or slime separator 20, such as, for example, of the Akins, Dorr, Hardinge or other suitable type. The separator 20 is here diagrammatically shown as comprising a tank 21, the bottom 22 of which is inclined upwardly to a discharge outlet 23. The heavy, desired particles settle to the bottom of the tank 21 while the slime or scuffings and other undesirable particles tend to float on top of the liquid in the tank. The material that settles to the bottom of the tank 21 is constantly urged toward the outlet 23 in any suitable way, as by means (not shown) of rakes, screws, or the like. Movement of the desired material to the discharge outlet 23 is somewhat impeded by the action of a counter stream of water issuing from a jet 24, and the counter-current thus provided carries the slime and scuffings and other rejects to an outlet 25. The outlet 25 maintains a constant liquid level in the tank 21, the overflow liquid together with the rejects carried thereby being discharged through the outlet 25 into a receptacle 26 if desired. While the particles discharged into the receptacle 26 have been termed rejects, it will be understood that under some conditions these particles may also have value, for purposes other than the particles discharged from the outlet 23.

It will be evident that the dispersing agent hereinbefore referred to serves the twofold purpose of enabling easy and efficient separation of the desired particles from the foreign matter in the separator 20, and of promoting self-attrition of the particles in the mill 14.

From the outlet 23 of the separator 20 the material may pass by way of a conduit 27 to any other apparatus which may be desired for further treatment of the material, and the material is eventually dried.

If desired, approximately one-half, or any selected suitable fraction of the material discharged from the outlet 23 of the separator 20 may be returned to the mill 14, and this is diagrammatically indicated by a conduit 28, here shown as receiving material from the outlet 23 and carrying it, as indicated by the arrows, to the hopper 10. Introduction into the mill 14 of scuffed, washed particles along with unscuffed particles promotes and scuffing in the mill of the unscuffed particles. When recirculation of material is

started, the feed to the mill is increased and the discharge is increased, inasmuch as the level in the mill is quite constant. By reason of recirculation of washed material the amount of dirt in the mill is in lower ratio to the contents. Inasmuch as the previously washed material becomes admixed with the new material, it has on the average the result of reducing the time inversely to the amount of material recirculated. Of course, previously scuffed and washed material is scuffed again with unscuffed material so that on the average all of the particles receive about the same amount of scuffing obtained by dividing the residual mill charge by the original hourly feed rate.

As already referred to herein above, one preferred use of my invention is in the treatment of zircon sand, which comprises zircon crystals lying for the most part between 60 and 150 mesh. Zircon which has been treated in accordance with my invention has exceptionally high resistance to the passage of current at elevated temperatures, and hence is particularly desirable for use as refractory electrical insulating material. Zircon is usually marketed as a concentrate from beach sands. Zircon concentrate is produced from beach sands which contain commercial quantities, by hydraulic and magnetic treatment for the removal of silica and other light silicates and for the removal of ilmenite with which it is associated. The zircon sand may also have been treated by flotation, for removal of rutile with which it is associated, and in that case the particles of zircon are covered with a film of flotation re-agents, such as oils, greases, acids, etc. which are not only difficult to remove but tend to collect other matter as a coating and fix it to the zircon grain. Furthermore, it is believed that zircon crystals subjected to the action of sea water for long periods become covered with a coating or film of one kind or another, either mechanically or of a chemically precipitated nature, or both. It is possible that, from the sea water, a certain absorption of the alkali or metal halides, or both, takes place on the surface of the zircon. In the case of some kinds of films, such as iron oxide films, the coating is visible, but often the coating is not subject to visual estimation either quantitatively or qualitatively. I have found through extended research that while some of these coatings are acid soluble or soluble in alkalis, or, in the case of flotation products, are soluble in commercial solvents, the electrical resistivity of a mass of particles so cleaned is often reduced instead of increased owing to some further phenomena brought about by the chemical cleaning agent or solvent. In the solution of this problem, I have determined that the slow gentle mechanical attrition of the surfaces of the particles, in water alone, produces zircon which shows electrical resistivity, measured through a compacted mass of grain at a temperature of 1600° F., at least three times greater than zircon cleaned by simple washing. Furthermore, when the slow gentle mechanical attrition is carried out under conditions which free the particles from the matter removed, as in the presence of a dispersing agent, as hereinbefore referred to, the zircon so treated shows electrical resistivity, measured through a compacted mass of grain at a temperature of 1600° F., at least 7 times greater than zircon cleaned by simple washing. In addition, whereas different lots of similar zircon of untreated grain varied in electrical resistance value over wide ranges, the grain produced from

treated zircon maintained a high average resistance. In the treatment of zircon for electrical purposes, in accordance with my invention, I prefer to use ammonia as a dispersing agent, as it is a carbon-free and a metal-free base, but I do not limit myself to this dispersing agent, as other dispersing agents of similar quality may be substituted. In the case of producing grain zircon for mechanical uses which demand the properties of zircon alone without interference by possible fluxing properties of coating materials, dispersing agents may be chosen on a basis of desired results as to mechanical cleanliness.

From the foregoing it will be apparent to those skilled in the art that the illustrated embodiment of my invention provides a new and improved method of treating materials, and accordingly, accomplishes the principal object of my invention. On the other hand, it also will be obvious to those skilled in the art that the illustrated embodiment of my invention may be variously changed and modified, or features thereof, singly or collectively, embodied in other combinations than those illustrated, without departing from the spirit of my invention, or sacrificing all of the advantages thereof, and that accordingly, the disclosure herein is illustrative only, and my invention is not limited thereto.

I claim:

1. The method of treating material particles comprising particles of refractory crystalline mineral material intended for use as electrical insulating material, which comprises, subjecting the particles to self attrition in the presence of a liquid containing a dispersing agent which is carbon-free and metal-free.

2. The method of cleaning discrete particles of hard crystalline mineral material, which comprises, charging a rotary tumbling mill so that the charge therein comprises only a liquid and the discrete particles, said liquid including a dispersing agent, causing the particles to be so tumbled in said mill that said particles constitute a substantially unitary tumbling mass, separating particles from cleanings, and returning a portion of said separated particles to mingle with the charge in said mill.

3. The method of cleaning discrete particles of crystalline mineral material comprising particles intended for use as electrical insulating material, which comprises, charging a rotary tumbling mill so that the charge therein comprises only a liquid and the discrete particles, causing the particles to be so tumbled in said mill that said particles constitute a substantially unitary tumbling mass, subjecting the material to a dispersing agent which is carbon-free and metal-free, and separating the particles from the cleanings.

4. The method of cleaning discrete particles of hard crystalline mineral material intended for use as electrical insulating material, which comprises, charging a rotary tumbling mill so that the charge therein comprises only a liquid and the discrete particles, said liquid including a dispersing agent which is carbon-free and metal-free, causing the particles to be so tumbled in said mill that said particles constitute a substantially unitary tumbling mass, separating particles from cleanings, and returning a portion of said separated particles to mingle with the charge in said mill.

5. The method of treating material particles, which comprises, in a prior stage subjecting a mass consisting of discrete particles of hard crystalline mineral material to self attrition only, in

the presence of water, subjecting the material to a dispersing agent, separating particles from cleanings, and returning a portion of said separated particles to mingle with particles being treated in said prior stage.

6. The method of treating material particles, which comprises, in a prior stage subjecting a mass consisting of discrete particles of hard crystalline mineral material to self attrition only, in the presence of water, subjecting the material to a dispersing agent while it is being subjected to self attrition, separating particles from cleanings, and returning a portion of said separated particles to mingle with particles being treated in said prior stage.

7. The method of removing foreign coatings from zircon grains to produce clean zircon grains for use in electrical refractory, which comprises, subjecting raw material consisting of discrete material particles comprising natural grain zircon to mutual rubbing action in the presence of water and in the absence of grinding bodies, treating the material with a dispersing agent which is carbon-free and metal-free, and separating the particles from the cleanings.

8. The method of removing foreign coatings from zircon grains to produce clean zircon grains for use in electrical refractory, which comprises, subjecting raw material consisting of discrete material particles comprising natural grain zircon to mutual rubbing action in the presence of water and in the absence of grinding bodies, treating the material with a dispersing agent which is carbon-free and metal-free, separating particles from cleanings, and returning a portion of said separated particles to mingle with particles being subjected to mutual rubbing action.

9. The method of removing foreign coatings from zircon grains to produce clean zircon grains for use in electrical refractory, which comprises, subjecting a mass consisting of discrete material particles comprising natural grain zircon to self attrition only, in the presence of water in a rotary tumbling mill, subjecting the material to a dispersing agent which is carbon-free and metal-free, and separating the particles from the cleanings.

10. The method of removing foreign coatings from zircon grains to produce clean zircon grains for use in electrical refractory, which comprises, subjecting a mass consisting of discrete material particles comprising natural grain zircon to self attrition only, in the presence of water in a rotary tumbling mill, said water containing a dispersing agent which is carbon-free and metal-free, separating particles from cleanings, and returning a portion of said separated particles to mingle with the particles in said mill.

11. The method of removing foreign coatings from discrete particles of hard crystalline mineral material to produce clean particles, which comprises, subjecting raw material consisting of such discrete particles to mutual rubbing action in the presence of water and in the absence of grinding bodies, treating the material with a dispersing agent, hydraulically separating particles from cleanings, and returning wet separated particles to mingle with particles being subjected to mutual rubbing action.

12. The method of removing foreign coatings from discrete particles of hard crystalline mineral material to produce clean particles, which comprises, subjecting raw material consisting of such discrete particles to mutual rubbing action in the presence of water and in the absence of

grinding bodies, said water containing a dispersing agent, hydraulically separating particles from cleanings, and returning wet separated particles to mingle with particles being subjected to mutual rubbing action.

13. The method of removing foreign coatings from zircon grains to produce clean zircon grains, which comprises, subjecting raw material consisting of discrete particles comprising natural grain zircon to mutual rubbing action in the presence of water and in the absence of grinding bodies, treating the material with a dispersing agent, hydraulically separating particles from cleanings, and returning wet separated particles to mingle with particles being subjected to mutual rubbing action.

14. The method of removing foreign coatings from zircon grains to produce clean zircon grains for use in electrical refractory, which comprises, subjecting raw material consisting of discrete material particles comprising natural grain zircon to mutual rubbing action in the presence of water and in the absence of grinding bodies, treating the material with a dispersing agent which is carbon-free and metal-free, hydraulically separating particles from cleanings, and returning wet separated particles to mingle with particles being subjected to mutual rubbing action.

15. The method of removing foreign coatings from zircon grains to produce clean zircon grains for use in electrical refractory, which comprises, subjecting a mass consisting of discrete material particles comprising natural grain zircon to self attrition only, in the presence of water in a rotary tumbling mill, said water containing a dispersing agent which is carbon-free and metal-free, separating particles from cleanings, and returning separated particles to mingle with the particles in said mill.

16. The method of cleaning discrete particles

of crystalline mineral material comprising particles intended for use as electrical insulating material, which comprises, charging a rotary tumbling mill so that the charge therein comprises only a liquid and the discrete particles, said liquid comprising a dispersing agent which is carbon-free and metal-free, causing the particles to be so tumbled in said mill that said particles constitute a substantially unitary tumbling mass, and separating the particles from the cleanings.

17. The method of removing foreign coatings from zircon grains to produce clean zircon grains for use in electrical refractory, which comprises, subjecting a mass consisting of discrete material particles comprising natural grain zircon to self attrition only, in the presence of water in a rotary tumbling mill, said water containing a dispersing agent which is carbon-free and metal-free, and separating the particles from the cleanings.

18. The method of removing foreign coatings from zircon grains to produce clean zircon grains, which comprises, subjecting raw material consisting of discrete particles comprising natural grain zircon to mutual rubbing action in the presence of water and in the absence of grinding bodies, said water containing a dispersing agent, hydraulically separating particles from cleanings, and returning wet separated particles to mingle with particles being subjected to mutual rubbing action.

19. The method of removing foreign coatings from zircon grains to produce clean zircon grains, which comprises, in a prior stage subjecting a mass consisting of discrete particles comprising natural grain zircon to self attrition only, in the presence of water, subjecting the material to a dispersing agent, separating particles from cleanings, and returning separated particles to mingle with particles being treated in said prior stage.

BASIL HORSFIELD.